

1

2,789,952

## COMPOUNDED TURBINE OIL

Troy L. Cantrell, Drexel Hill, Pa., and John G. Peters, Audubon, N. J., assignors to Gulf Oil Corporation, Pittsburgh, Pa., a corporation of Pennsylvania

No Drawing. Application August 19, 1954,  
Serial No. 451,041

1 Claim. (Cl. 252—32.7)

This invention relates to lubricating compositions and more particularly to steam turbine oils adapted to prevent rusting and corrosion of metal turbine parts which are exposed to moisture.

Various lubricating compositions have heretofore been disclosed for lubricating steam turbines but the prior compositions have not been entirely satisfactory. Some of the prior compositions have exhibited good resistance to oxidation but they have not given complete protection against rusting and corrosion of metal turbine parts which are exposed to moisture.

The present invention is based upon a particularly effective lubricating composition having good resistance to oxidation combined with good lubricating characteristics, and corrosion and rust-inhibiting properties.

The improved lubricating composition of this invention consists essentially of a homogeneous mixture of lubricating oil, a metal alkyl thiophosphate, an alkyl phenol and a substantially neutral addition product of isoamyl octyl acid phosphate with primary fatty amines containing from 8 to 18 carbon atoms. We have found that the three addition agents just mentioned cooperate to give a composition having excellent resistance to oxygen absorption and increased oxidation life. Furthermore the composition has good corrosion and rust-inhibiting properties. These rust-inhibiting properties are unexpected in view of the performance of the individual additives and of combinations of only two of the additives.

The lubricating oil to which the other constituents are added is advantageously a highly refined paraffinic oil. By the term "highly refined paraffinic oil" we mean a petroleum lubricating oil which has been refined by one of the more drastic refining methods known in the art, for example, by conventional aluminum chloride refining or by a solvent extraction adapted to remove all or substantially all of the unsaturated and naphthenic constituents of the oil. Aluminum chloride refined or solvent extracted paraffinic base oil, such as a Pennsylvania oil, provides an excellent base oil for the composition of the invention. However, drastically refined Mid-Continent and Gulf Coastal oil may also be used.

The metal alkyl thiophosphates which can be used in accordance with the invention are advantageously those whose metal component is a metal of group II of Mendeleff's periodic arrangement of the elements. Included within this group are magnesium, calcium, zinc, strontium, cadmium and barium. However, other metals including aluminum, copper, lead, tin, iron and manganese can also be employed. The alkyl substituents are preferably those containing between 3 and 12 carbon atoms. Examples of the alkyl groups which can be used are butyl, particularly tertiary butyl, amyl, isoamyl, tertiary amyl, hexyl, heptyl, octyl, nonyl, decyl, dodecyl and the like. While the mono-alkyl esters can be used, the di-alkyl esters are particularly suitable for the purposes of the invention. An example of a particularly effective compound which can be used is zinc dihexyl thiophosphate. When zinc dihexyl thiophosphate is used, it is preferably

2

used in an amount between about 0.01 and 0.1 percent by weight based on the weight of the total composition. An amount greater than about 0.1 percent is undesirable in that the neutralization number of the final product is increased above the maximum set for commercial use.

The alkyl phenol which is used in accordance with the invention is advantageously a di- or trialkylated phenol or cresol with at least one of the alkyl groups being a tertiary alkyl group. The alkyl groups are preferably those containing between 3 and 12 carbon atoms. Good results can be obtained with a tri-tertiary butyl phenol or a di-tertiary butyl cresol. Examples of the preferred alkylated phenols are 2,4,6-tri-tertiary-butylphenol, 2,6-di-tertiary-butyl-4-methylphenol and bis(2-hydroxy-3-tertiary-butyl-5-methylphenyl)methane. The alkyl phenols are advantageously used in amounts of about 0.1 to about 2.0 percent by weight based on the weight of the total composition.

The fatty amine salt of isoamyl octyl acid phosphate which can be used in accordance with the invention is prepared by reacting isoamyl octyl acid phosphate with a primary fatty amine containing from 8 to 18 carbon atoms. One example of a primary fatty amine suitable for the purpose of this invention is cocoamine, which is a commercially available product prepared by converting coconut oil fatty acids into the corresponding amine. It consists mostly of monolauryl amine with minor amounts of adjacent homologues. The cocoamine salt of isoamyl octyl acid phosphate and its preparation are fully described in U. S. Patent No. 2,371,851 which issued on March 20, 1945 to Herschel G. Smith and Troy L. Cantrell. As disclosed in said patent, the cocoamine salt of isoamyl octyl acid phosphate can be readily prepared by reacting cocoamine with isoamyl octyl acid phosphate in approximately equimolecular ratios, the reaction being so controlled as to produce substantially neutral reaction mixtures having a pH value within the range 5.5 to 7.5, as illustrated in Examples 1 and 2 of that patent. The isoamyl octyl acid phosphate employed is a di-ester of ortho-phosphoric acid having the following formula:



45 This compound is also known as 3-methylbutyl, 2-ethylhexyl acid orthophosphate. It readily reacts with cocoamine and other primary fatty amines containing from 8 to 18 carbon atoms. Instead of cocoamine we can use other primary fatty amines containing from 8 to 18 carbon atoms. These amines include mono-capryl,



55 mono-lauryl, mono-myristyl, mono-palmityl and mono-stearyl amines. The fatty acid amine salt of isoamyl octyl acid phosphate is preferably used in an amount between about 0.01 and about 1.0 percent by weight based on the weight of the total composition.

60 The lubricating oil compositions of this invention can contain other additive agents, if desired, to improve other specific properties without deleteriously affecting the beneficial properties of the compositions. For example, pour point depressors, viscosity and viscosity index improvers, dyes, sludge inhibitors and the like can be used. Also, if desired, the oil can contain a foam inhibitor such as organo-silicon oxide condensation products, organo-silanol condensation products, and the like.

65 The individual constituents of compositions of this invention may be added to the lubricating oil base in either order or simultaneously, either *per se*, or in the form of a mineral oil concentrate. The latter practice is some-

times desirable in order to facilitate compounding of the lubricating oil.

0.0033 percent by weight of Dow-Corning silicone fluid 200 as a foam inhibitor. The results were as follows:

| Composition, percent by wt.....                            | A               | B               | C               | D               | E           |
|------------------------------------------------------------|-----------------|-----------------|-----------------|-----------------|-------------|
| Base oil.....                                              | 98.75.....      | 99.9.....       | 99.96.....      | 99.16.....      | 98.63.....  |
| 2,6-di-tertiary-butyl-4-methylphenol.....                  | 1.25.....       | .....           | .....           | 0.8.....        | 1.25.....   |
| Zinc dihexyl thiophosphate.....                            | .....           | 0.1.....        | .....           | .....           | 0.1.....    |
| Cocoamine isoamyl octyl orthophosphate.....                | .....           | .....           | 0.04.....       | 0.04.....       | 0.02.....   |
| Amount of rust, ASTM D 943-47 T, 500 hours, iron coil..... | Heavy rust..... | Heavy rust..... | Heavy rust..... | Heavy rust..... | Bright..... |

The advantages obtained by the use of the improved lubricating composition of the invention as compared with the use of similar compositions containing only one or two of the three addition agents are illustrated in the following specific examples. The effectiveness of the rust-inhibiting properties has been demonstrated by subjecting the lubricating compositions to the procedure of ASTM test D 943-47 T. Briefly, this test is carried out by passing oxygen at a measured rate of 3 liters per hour into an oil-water mixture maintained at 203° F. and having an iron coil immersed therein. According to the procedure followed herein, the test was carried out for 500 hours. The corrosion-inhibiting properties of the compositions were determined by examining the iron coil before and after completion of the test. The amount of rust on the coil was thus used to determine the effectiveness of the composition in preventing rust.

To illustrate the rust-inhibiting properties of the composition of the invention as compared with similar compositions containing only one or two of the addition agents, samples of the oils were subjected to the above-described ASTM test D 943-47 T. The base oil used in the test was a highly refined, aluminum chloride treated, paraffinic turbine oil stock having an API gravity between about 30.5° and 32.5° and a viscosity of about 150 SUS at 100° F. In each instance the oil also contained

As can be noted from the above data, a composition of the invention, composition E, is strikingly superior to compositions not within the scope of the invention. The synergistic effect obtained is shown inasmuch as the individual additives and a combination of only two of the additives did not give the improved result obtained by a combination of all three of the additives.

While the invention has been described above with reference to certain specific embodiments thereof by way of illustration, it is to be understood that the invention is not limited to such embodiments except as hereinafter defined in the appended claim.

We claim:

A rust-inhibiting oil consisting essentially of a major proportion of a mineral lubricating oil and minor proportions consisting of about 0.1 to about 2.0 percent by weight of 2,6-di-tertiary-butyl-4-methylphenol, about 0.01 to about 0.1 percent by weight of zinc dihexyl thiophosphate and about 0.01 to about 1.0 percent by weight of the cocoamine salt of 3-methylbutyl,2-ethylhexyl acid orthophosphate.

References Cited in the file of this patent

UNITED STATES PATENTS

2,364,283 Freuler ..... Dec. 5, 1944  
2,371,655 Smith et al. ..... Mar. 20, 1945